

## UNITED STATES PATENT OFFICE

1,973,612

## METHOD OF SECURING DURABLE ADHESIONS OF LIQUID COATINGS TO ZINC SURFACES

Milford H. Corbin, Chicago, Ill., assignor to Ault &amp; Wiborg Corporation, a corporation of Ohio

No Drawing. Application January 16, 1931,  
Serial No. 509,275

2 Claims. (Cl. 91—68)

This invention relates to a method of applying paints to zinc or zinc surfaced materials so that the paints will adhere to such surfaces. Metals of the zinc type appear to be somewhat peculiar among metals in that the paints or lacquers which are applied to surfaces of such metals become very short or brittle and crack or peel from the metal. If an oil-base material is used, zinc seems to accelerate the polymerization so that the paint does not long adhere, or if a pyroxylin-base material is used, the presence of the zinc seems to break it down. These difficulties have tended to limit the fields of usage of zinc and zinc coated materials.

15 The object of the invention is to provide a method of causing paints, enamels or lacquers, whether of an oil-base type or pyroxylin-base type, to adhere to zinc or zinc coated materials as the materials would do to ordinary metals.

20 The invention is predicated upon the discovery that this harmful affectation of the paint or enamel or lacquer by the zinc is strictly interface phenomena and that either a thin coverage of the zinc surface with another metal or the displacement of the zinc at the surface by other metals, provides a surface to which the paints or lacquers or enamels will adhere without deterioration.

For instance, the liquid coatings can be made 30 to adhere to the zinc by electroplating a thin layer over the zinc of some other metal such as copper or nickel. The preferred method of this invention, however, is to displace zinc molecules at the surface and substitute for them other 35 molecules which provide a surface to which the paints or the like will adhere without deterioration. This is accomplished by dipping the zinc in or contacting the zinc with a solution including salts of metals which interchange with the zinc 40 due to the difference in electric potential between the metal ions and the zinc. Though many such solutions are possible I find that the invention is well exemplified by the use of nickel. For instance, a solution of nickel chloride and 45 ammonium chloride will deposit a nickel film on the zinc when brought into contact with the zinc.

After the contacting, whether by immersion or otherwise, the surface is preferably washed and dried, after which paints, lacquers and enamels 50 will readily adhere to it and will not deteriorate any more rapidly than on ordinary materials.

A still better surface is obtained by adding sodium thiocyanate to the solution as this results in the deposit on the zinc surface of both 55 the nickel and nickel sulphide. A small amount

of zinc chloride in the solution aids this deposition when the solution is new, though additional amounts need not be added during the continued use of the solution due to the fact that additional quantities are formed in the use of the solution.

A typical formula is as follows:

6 oz. NH<sub>4</sub>CL,  
4 oz. NiCl<sub>2</sub>,  
2 oz. NaCNS,  
1/2 oz. ZnCl<sub>2</sub>,  
1 gallon H<sub>2</sub>O.

A sulphate solution of salts including nickel salts, likewise provides a modification of the zinc surface of the same nature. A sulphate type bath should include nickel sulphate, a small quantity of zinc sulphate, sodium thiocyanate, and sodium acetate. A typical formula for sulphate baths is as follows:

12 oz. NiSO<sub>4</sub>,  
3 oz. NaCNS,  
1 oz. NaC<sub>2</sub>H<sub>3</sub>O<sub>2</sub>,  
4 1/2 oz. ZnSO<sub>4</sub>,  
1 gal. H<sub>2</sub>O.

In practice, the zinc is usually dipped in the treating solution for one-half minute at a temperature of 100° F., after which it is washed and dried.

While this disclosure has been made chiefly in relation to zinc and oil-base or pyroxylin coating materials, it is adaptable for use in all cases where a specific coating material will not adhere to a specific metal as it will be readily understood by the skilled in the art that by selecting a solution of a salt of a metal having a potential different from that of the metal to be treated, (in the nature of the potential difference between zinc and the nickel salt solution), the replacement of surface molecules can be accomplished to inhibit the specific catalytic action which the surface of the metal in question may have upon the specific liquid coating to be applied to it.

Having described the invention, I desire to be limited only by the ensuing claims:

1. A method of preventing the deterioration of lacquers of the oil-base or pyroxylin type when said lacquers are applied to zinc surfaces, said method comprising the treatment of zinc surfaces, before lacquering, with an aqueous solution containing an inorganic salt of nickel and a water soluble sulphur containing compound, whereby the surface molecules of zinc are re-

15

70

75

80

85

90

95

100

115

placed with surface molecules of nickel and nickel sulfide which will protect the lacquer from being deteriorated by the zinc surface.

2. A method of preventing the deterioration of 5 lacquers of the oil-base or pyroxylin-base type when said lacquers are applied to zinc surfaces, said method comprising the treatment of zinc surfaces, before lacquering, with an aqueous solu-

tion containing, in one gallon of water, 6 oz. ammonium chloride, 4 oz. nickel chloride, 2 oz. sodium thiocyanate and  $\frac{1}{2}$  oz. zinc chloride, whereby the surface molecules of zinc are replaced with surface molecules of nickel and nickel sulfide which will prevent the lacquer from being deteriorated by the zinc surface.

MILFORD H. CORBIN.

85

10

15

90

20

95

25

100

30

105

35

110

40

115

45

120

50

125

55

130

60

135

65

140

70

145

75

150